

## UNITED STATES PATENT OFFICE

RUSSELL H. McCARROLL AND GOSTA VENNERHOLM, OF DEARBORN, MICHIGAN, ASSIGNEES TO FORD MOTOR COMPANY, OF DEARBORN, MICHIGAN, A CORPORATION OF DELAWARE

## METHOD OF MANUFACTURING CAST IRON, AND CAST IRON ARTICLES

No Drawing.

Application filed January 19, 1931. Serial No. 509,879.

This invention relates to the manufacture of cast iron articles and particularly to sand cast iron and has for its principal object to provide a new article of manufacture of cast iron and a new and improved manufacturing method therefor, including the preparation of an iron of a predetermined analysis and a treating of the same to secure a product of unusually high physical properties, heretofore not thought possible in cast iron.

The product heretofore resulting from the casting of iron is gray cast iron, mottled cast iron, and white cast iron, depending upon such factors as the analysis of the iron, the process of melting, and the rate of cooling. The most important of these irons are the gray cast and white cast iron. Gray cast iron is characterized by the presence of carbon interspersed throughout the matrix in the form of graphitic flakes or fissures, while in white cast iron the carbon is in the combined state, that is, in the form of iron carbide and as a solid solution of iron and iron carbide.

White cast iron is extremely hard and very brittle and because of the difficulty of machining it by the ordinary methods its usefulness is very limited. Considerable amounts of white cast iron, however, are employed for the production of malleableized iron, the latter being soft and ductile and of relatively low strength, compared with steel.

It is a matter of common knowledge that gray cast iron, although used extensively in the industries, is of relatively low tensile strength and that it is not possible, although the matrix of gray iron is of essentially the same composition as steel, appreciably to improve the physical properties of gray cast iron by the common and well known hardening and tempering heat treatments that are effectively employed for the treatment of steel. This is mainly due to the presence of the graphitic flakes and fissures which in all cases form planes of weakness. It is, however, possible to improve the physical properties of gray cast iron by special methods of treatment. As far as we are aware the only methods heretofore commercially used, particularly in connection with the production of sand cast iron are what are known as the

superheating method and the mold heating method. In the superheating, the molten iron is heated considerably above the temperatures ordinarily employed in the furnace, the object being to increase solubility for carbon and as a result of such increased solubility the final product contains its free carbon in the form of smaller graphitic flakes and fissures than is present in the common gray cast iron. While the superheating method results in securing an improved iron, this method of treatment is subject to the objections that the product still contains graphitic flakes and fissures in an extent sufficient to have a weakening effect, and that the higher temperatures necessary involve greater production costs because of the increased furnace maintenance costs.

The second method, namely, the mold heating method, consists in heating the molds before the molten iron is poured therein and in employing an iron of an analysis that would, if cast into unheated molds, result in the production of white or mottled cast iron. The pre-heating of the molds insures a slow rate of cooling, prevents white cast iron from freezing out, should the analysis be such as would ordinarily form such iron, and results in producing an iron having a pearlitic matrix with free carbon distributed through such matrix as graphitic flakes. This method is subject to the objection noted above with respect to the formation of graphitic flakes and fissures and is also subject to the objection of increased production costs and difficulties in handling the heated molds.

We aim by the present invention to produce as a final product an iron free from graphitic flakes and fissures with the free carbon in the form of temper carbon and with the remainder of the carbon in a state corresponding to that found in the transformations, pearlite, sorbite, troosite or martensite, depending upon the uses for which the product is intended. The present invention may be briefly said to depend upon a predetermined analysis of the iron, the constituents thereof falling within fairly well defined limits, and, in conjunction with such analysis, a heat treatment of the iron after casting

so as to control the decomposition of the carbon content. The method hereinafter to be more fully described is particularly applicable to casting in sand molds although the invention is not limited to the use of any particular type of molds.

We have found that an iron, whose constituents fall within the following limits, when subjected to the heat treatment herein-  
10 after to be described, will have the desired high physical properties which it is the object of the present invention to obtain:

Carbon from 1.90 to 2.30%  
15 Manganese from .20 to .65%  
Silicon from 1.50 to 2.20%  
Phosphorus below .12% and  
Sulphur below .12%.

An iron of the following analysis prepared  
20 in accordance with the invention has given highly successful commercial results:

25 Carbon 2.08%  
Manganese .21%  
Silicon 1.85%  
Phosphorus .05% and  
Sulphur .06%.

Molten metal of the above described analysis is cast, preferably in sand molds, to secure an article, or articles, of the predetermined desired shape and size. Due to the analysis, the casting produced is mainly white iron. After the casting has cooled it is then reheated to above the critical range, for example, up to approximately 1750° F., followed by various types of cooling treatment depending upon the matrix composition desired as set forth above. The result of this treatment is to give a solid solution, eutectoid or intermediate, matrix with the free carbon in the form of temper carbon. The time of heat treatment will depend upon the cross section of the casting. For castings up to one-half inch cross sectional dimensions, a heat treatment at the maximum temperature of one and a half hours duration has been found to be sufficient.

In some cases the castings are then reheated to a temperature just slightly below the critical range and are allowed to air cool, to insure a matrix which is mainly pearlite (and sorbite) in which is imbedded free particles of temper carbon.

The product resulting from the above described method that is with an iron of approximately 2% carbon, is found to have its carbon content distributed approximately 1% in the form of a combined carbon, that is, iron carbide free in solid solution in the matrix, or eutectoid and approximately 1% in the form of free temper carbon interspersed throughout the matrix. This product has remarkably high physical properties, giving on test a tensile strength of over 90,000

10 pounds; the hardness of the product is readily controllable as desired.

It will be understood however that the ratios of carbon distribution in the forms of temper carbon and in solution as iron carbide will vary according to the analysis of the batch. It will further be understood that such analysis as well as the heat treatment may be varied from the specific example above described and that such changes, variations and modifications as may be resorted to without departing from the basic underlying principles of the invention are intended to be covered by the claims hereunto appended.

80 We claim:

1. The method of manufacturing cast iron which consists of preparing a batch of molten metal in which the constituents will be within the following limits:

85 Carbon from 1.90 to 2.30%  
Manganese from .20 to .65%  
Silicon from 1.50 to 2.20%  
Phosphorus below .12% and  
Sulphur below .12%,

90 casting the molten metal in a mold to secure an article of predetermined configuration, and after the article has cooled reheating to approximately 1750° F. for a predetermined period of time, depending upon cross section and analysis, sufficient to decompose the combined carbon, then lowering the temperature to a point somewhat above the critical range, and preventing further decomposition at such point by a rapid cooling, such as quenching, thereby to obtain a matrix composed of solid solution, and then finally reheating to a point below the critical range, to produce a matrix composed of martensite, troostite, sorbite or pearlite as determined by the reheating temperature.

95 2. As an article of manufacture, heat treated cast iron having a composition within the following limits:

100 Carbon from 1.90 to 2.30%  
Manganese from .20 to .65%  
Silicon from 1.50 to 2.20%  
Phosphorus below .12% and  
Sulphur below .12%,

105 free from graphitic flakes and fissures in which the carbon content is substantially equally distributed as solid solution in the matrix and throughout the matrix as temper carbon.

110 In testimony whereof we affix our signatures hereto.

115 RUSSELL H. McCARROLL.  
GOSTA VENNERHOLM.

120 125

130